

## UNITED STATES PATENT OFFICE

ERIC WAHLFORSS, OF ST. CLOUD, MINNESOTA, ASSIGNOR, BY MESNE ASSIGNMENTS,  
TO ARTHUR D. LITTLE INDUSTRIAL CORPORATION, OF NEW YORK, N. Y., A COR-  
PORATION OF DELAWARE

## PROCESS FOR THE MANUFACTURE OF PAPER PULP

No Drawing.

Application filed July 30, 1926. Serial No. 126,087.

The present invention relates to a new and improved process for the production of paper pulp from hard woods, together with the product resulting from such a process.

According to existing practice, pulp for paper-making purposes is ordinarily prepared either mechanically or chemically. In the mechanical method the wood ordinarily soft or coniferous is reduced to a finely divided form suitable for the paper-making operation by grinding. Although this method has certain advantages from the standpoint of cost and is quite commonly employed in large scale production for the manufacture of newsprint and similar forms of paper, nevertheless it does result in a perceptible shortening of the cellulose fibres with a resultant impairment in strength of the finished paper. In the chemical method the organic encrusting substances other than the cellulose fibres are substantially completely removed from the natural wood through the use of chemical reagents. The cellulose fibres thus freed from surrounding encrustations are then adapted for the subsequent paper-making operations. It is impossible to control the chemical method of digesting the natural wood with sufficient accuracy to insure the removal of all of the organic encrusting substances without also digesting a certain percentage of the cellulose fibre. In consequence, the resulting pulp not only loses a certain percentage of cellulose fibre initially present but is weakened, due to impairment in strength of the remaining fibre as a result of the digesting. According to the Kraft process so-called, the cooking or digesting of the natural wood with chemical reagents is halted before the ligneous and intercellular materials have been completely removed and insuring that all of the cellulose fibre originally present in the wood is retained. The pulp obtained by virtue of this process is darkened somewhat by the presence of a residue of organic material, but contains all of the cellulose fibre in substantially its initial volume and strength.

In addition to these methods commonly employed for the production of paper pulp, it has been suggested that both the chemical

and mechanical methods of preparing the pulp be preceded by treatment with steam or hot water to soften the wood and facilitate the subsequent grinding or chemical operations. These suggestions are also intended to permit the use of certain resinous woods not otherwise capable of satisfactory employment for the production of pulp for paper-making purposes. Where this result is intended, the pre-cooking with steam is designed to remove the resins and similar materials from coniferous woods in order to enable this type of wood to be successfully reduced to a pulp by the usual chemical operation.

I have discovered that it is possible to produce a grade of pulp from hard wood well suited for certain types of paper products without resorting to mechanical grinding of the raw material or the use of added chemical reagents. This pulp may be introduced directly into the usual paper-making process without further treatment, and as an example may be employed either alone or in admixture with kraft pulp in the field in which kraft is now commonly used. I accomplish the desired result by converting the organic, encrusting substances surrounding the fibre of the hard wood into a condition sufficiently plastic to permit displacement and separation of the fibres without grinding or further chemical treatment. The product resulting from this conversion of the organic encrusting substances is essentially different from the product resulting from existing methods, in which the organic substances are either broken down by mechanical action or dissolved and removed by chemical action. Under certain conditions it may be desirable, although not essential, to treat the product resulting from my process by impact in a ball mill or rod mill for the purpose of further displacing and separating the fibre bundle. I have found that the desired result can be satisfactorily attained by treating the raw material under pressure with certain volatile substances and organic compounds extracted directly from the material itself. To this end the wood is initially subjected to the action of water or water vapor at a substantial tem-

55

60

65

70

75

80

85

90

95

100

perature and pressure, the operation being carried out in a substantially closed chamber to retain and utilize the beneficial action of the volatile and organic substances progressively extracted from the wood. In actual practice I have found that the operation may be satisfactorily carried out in a closed chamber at pressures of 75 to 100 pounds for a period approximating two hours, and at a 10 temperature corresponding to the temperature of steam at the given pressure. Although this relatively high pressure is desirable, nevertheless experiments have indicated that lower pressures with a longer period of treatment may suffice to accomplish the desired result, and accordingly my invention contemplates the treatment of the raw material under pressures and temperatures and for a sufficient period of time to obtain the desired plastic 15 condition of the organic, encrusting substances without charring the wood or substantially breaking down the cellulose fibres. At the completion of this operation the resulting fibrous material may be subjected to an impact 20 operation of the character performed in a ball or rod mill, and thereafter converted into paper in the usual manner.

Under certain circumstances it may be desirable to utilize the liquor resulting from 30 the treatment of the raw material in subsequent operations, and with this in mind I propose to save the liquor after the removal of the pulpy mass and use this liquor with the addition of whatever water may be necessary 35 for the treatment of the next succeeding batch of wood. It is my belief that up to a certain point the increasing strength of the liquor resulting from the extraction of certain volatile and organic substances from the 40 wood will facilitate subsequent operations. However, although the reuse of this liquor is desirable, it is nevertheless not essential to the proper functioning of my process.

In the actual practice of my process I have 45 immersed hard wood in the form of chips in a closed vessel or chamber in the presence of water without the addition of chemical reagents. The temperature of the water and wood is then elevated through the application 50 of external heat until a pressure of 100 pounds is obtained within the chamber. This pressure is maintained through proper control of the heat for a period approximating two hours without permitting the escape of 55 any substantial quantity of vapor from within the chamber. At the completion of the operation, the hard, brittle, encrusting substances have been reduced to a soft and relatively plastic mass which permits further 60 separation and displacement of the fibre bundle by a simple impact operation.

I consider that without grinding or digesting with added chemical reagents I have 65 been able to produce a new substance adaptable for use directly in the paper-making

operation in the same fashion as existing forms of paper pulp.

The substances present in the natural wood may be generally classified as organic materials, and I believe that in the practice of my process the cooking of the wood in the presence of water gradually develops or releases the volatile, organic materials which in turn react upon and soften the normally hard encrusting substances. Although a 70 certain percentage of these encrusting substances may be removed from the resulting pulp, nevertheless I have demonstrated by actual experiment that the major portion of these encrusting substances remain in the 80 pulp.

What is claimed is:

1. The process of producing paper pulp from hardwood in chip or similar form which consists in converting the organic encrusting substances initially present in the hardwood into a condition sufficiently plastic to permit spreading and separation of the individual fibres without material disintegration of the fibres and while still surrounded by the major portion of the encrusting substances, and thereafter removing and subjecting the softened fibrous mass to an impact or like operation to further complete the preparation of pulp for paper 95 making purposes.

2. The process of producing paper pulp from hardwood in chip or similar form which consists in subjecting the wood to the action of organic compounds derived from the hardwood itself when heated in the presence of water to a temperature corresponding to a steam pressure in approximately the range of from 75 to 100 pounds until the organic encrusting substances contained in the hardwood are softened and rendered plastic and the fibrous mass capable of further separation and conversion into pulp without chemical treatment or mechanical pulp grinding.

3. The process of producing paper pulp from hardwood in chip or similar form which consists in subjecting the hardwood under heat and pressure to the action of organic compounds derived from the wood itself in heating the wood in the presence of water to temperatures corresponding to steam pressures, ranging approximately from 75 to 100 pounds, to soften and render plastic the organic encrusting substances contained in the hardwood without change or material disintegration of the fibres themselves, removing the fibrous mass from the resulting liquor, and reusing the liquor for the next 115 succeeding batch.

4. A material prepared from hardwood and suitable for the production of pulp for paper products, consisting of hardwood fibres having the length in which the fibres naturally occur substantially unshortened by 130

chemical or mechanical action and surrounded by the major portion of the organic encrusting substances originally present in the wood but softened and rendered plastic  
5 throughout in a manner to permit complete separation of the individual fibres without grinding or similarly treating the material, the material having substantially the physical shape and configuration of chip or like  
10 form in which cut from the natural wood and a characteristic dark-brown color resulting from the interaction of constituents present in the wood but being entirely free of chemicals or compounds resulting from  
15 chemical constituents other than those originally present in the wood.

5. The process of producing pulp suitable for paper makers' purposes from hardwood in chip or similar form which consists in immersing the wood in water in a substantially closed chamber, supplying heat to create a pressure within the chamber in the approximate range of from 75 to 100 pounds, continuing the application of heat for a sufficient  
20 25 period to soften the organic encrusting materials and leave the fibrous structure substantially intact, and thereafter converting the fibrous mass to pulp for paper makers' purposes by an impact or similar non-grinding action.

ERIC WAHLFORSS.

35

40

45

50

55

60

65